

1,158,318.

H. E. SHELDON.  
INGOT MOLD.  
APPLICATION FILED MAR. 30, 1912.

Patented Oct. 26, 1915.

FIG. 1



FIG. 2



WITNESSES.

Robert C. Totten  
J. R. Keller

INVENTOR.

H. E. Sheldon  
By May C. Totten  
Attest

# UNITED STATES PATENT OFFICE.

HARRY E. SHELDON, OF PITTSBURGH, PENNSYLVANIA.

## INGOT-MOLD.

1,158,318.

Specification of Letters Patent.

Patented Oct. 26, 1915.

Application filed March 30, 1912. Serial No. 687,366.

To all whom it may concern:

Be it known that I, HARRY E. SHELDON, a citizen of the United States, and resident of Pittsburgh, in the county of Allegheny and State of Pennsylvania, have invented a new and useful Improvement in Ingot-Molds; and I do hereby declare the following to be a full, clear, and exact description thereof.

10 My invention relates to an ingot mold for casting steel ingots, its object being to provide an ingot mold of longer life than the cast iron molds now in universal use.

It is well known that cast iron ingot molds 15 are short lived by reason of the recesses or cavities which appear in the inner surfaces, particularly in the lower portion thereof, and more particularly within two feet of the bottom of the mold. The molten metal 20 supplied to the mold during the casting of the ingot enters within these recesses or cavities and upon solidification locks the ingot in the mold so that it cannot be stripped therefrom thereby necessitating 25 the destruction of the mold; these ingot molds having an average life of only about sixty heats. I have discovered that these cavities in the molds are not, to any appreciable extent, due to the abrasion produced

30 by the stripping of the ingots from the molds, but are due to a phenomenon akin to osmotic action. This action can be described as follows: The cast iron ingot molds are relatively high in carbon, and may 35 be higher in manganese sulfur phosphorus and other impurities than the molten steel; and a large portion of the carbon in such cast metal appears as free carbon, not being chemically united with the iron. The

40 molten steel cast therein is of course much purer than this cast iron, having only a relatively small proportion of carbon or other impurities chemically united with the iron of the steel body. When this steel in

45 a highly molten condition is poured within the cold cast iron mold, the latter does not melt and so mix with the molten steel or dissolve gradually from the face of the mold, but the molten steel which is com-

50 posed of a more dilute alloy, infuses itself or immigrates into the higher alloy and causes, or tends to cause, an increase in the size and dilution of the higher alloy until both alloys are of the same composition,

55 there being a sharp separation between the higher alloy, or cast iron, and the lower

alloy, or molten steel, which envelops it. During this infusion or immigration of the steel into the cast iron, globules or fragments of the cast iron separate therefrom 60 and continue to be acted on by the molten steel or lower alloy in the same fashion as is above described with reference to the parent mass of the cast iron or higher alloy, and in this way the globules or fragments are, as 65 it were, dissolved within the molten steel or lower alloy. If the infusion or immigration of the molten steel into the cast iron be checked, as by the solidification of the metal, at any stage previous to complete merger of 70 the two metals or alloys, the remaining globules or fragments, if any, of the cast iron or higher alloy separated from the mold body, will remain as hard spots in the mass of the steel or lower alloy. I have 75 found that such infusion or immigration of the molten steel acts upon the walls of the cast iron molds and is responsible for the attack of the former upon the latter, causing the recesses or cavities in the inner mold 80 faces hereinbefore referred to, and the appearance of the hard spots in the sheets, plates or other products made from the ingots.

I have discovered that, if the mold wall 85 is of approximately the same composition as the metal poured into the mold, osmotic infusion or immigration of the poured metal in the mold wall does not take place, and consequently the formation of cavities with- 90 in the mold walls and hard spots in the ingots are practically overcome, and the life of the mold is prolonged and the quality of the metal cast is greatly improved.

My invention therefore consists, generally 95 stated, in an integral mold for casting steel ingots formed of cast steel; and in such mold formed of steel having approximately the same carbon content or content of other impurities as that of the steel to be cast 100 therein.

The particular method of operation herein disclosed is not claimed in this application inasmuch as it forms the subject matter of applicant's co-pending application No. 105 687,365.

In the accompanying drawing Figure 1 is a perspective view of one form of ingot mold embodying the invention; and Fig. 2 is a 110 sectional view of the same.

The ingot molds embodying the invention are formed of cast steel, for example, either

Bessemer steel or open hearth steel, and are formed as integral castings in the ordinary way of forming steel castings. They can be formed in the steel making plant where they 5 are to be used and are thus easily formed of the same or approximately the same carbon content as the steel produced in the plant.

In the accompanying drawing I have illustrated the ingot mold 2 resting on the 10 bottom plate or casting stand 3 and the metal can be poured into the ingot mold either through the top opening 4 thereof or from below, for example, through the runner 5 which has side runners 6 leading 15 to different ingot molds and communicating with the base thereof. In the forming of the steel ingot molds the most satisfactory results have been secured where the steel in the mold contains from .20 to .30 20 per cent. of carbon, the amount of manganese, phosphorus and sulfur present being within reasonable commercial limits.

To adapt the steel ingot molds for the casting of all characters of steel, however, 25 they should not have a carbon content of over two per cent. When there is no greater difference in proportion of impurity or alloy in the metal than is found between the ordinary molten steel cast in ingots and a steel 30 mold having this proportion, such so called osmotic action is practically overcome. In like manner the other impurities generally present in steel should be within the same practical working limit, the percentage of 35 manganese not being over two per cent. and the percentage of sulfur and phosphorus not being higher than in steel containing such proportions of impurities. Within such limits I practically prevent such osmotic infusion or immigration of the poured steel 40 into the walls of the mold, and thereby prevent the formation of cavities in the mold walls, and the appearance in the ingot of the hard spots formed from portions of the 45 mold walls detached as a result of such infusion or immigration, as above described. I always prefer, however, to employ a mold formed of steel within, say, 10 or 20 points of carbon content of the actual steel to be 50 cast in the mold, so that all tendency to this osmotic action between the steel and the mold body shall be eliminated.

Another advantage obtained from the invention is that in the use of the cast steel 55 molds in casting the steel ingots, the body of the mold is never raised to anything approximating the melting point of the metal of which it is composed. For example, the

melting point of cast iron is approximately from 2200 to 2300° F.; and the heat of 60 ordinary soft cast steel when being poured is in the neighborhood of 2700 to 2800°. In casting the ingots in cast iron molds the heat of the molten metal is quickly taken up by the mold which is raised to a temperature of 65 from 1200 to 1400°, about two-thirds of the melting point of the mold metal. This heating up of the mold close to its melting point naturally leads to disintegration and aids in the gradual cutting out of particles or 70 portions of the mold body. In use of the steel ingot molds, however, while they may absorb about the same heat from the body of the metal, the mold is only raised to about one-half of its melting temperature, and 75 such disintegration is therefore naturally resisted. Practical use of molds made in accordance with the present invention proves that they outlast the cast iron molds many times, the limit of wear not having yet been 80 ascertained.

The inner faces of the molds remain smooth and practically solid without any substantial indication of the formation of recesses or cavities which when solidified 85 would lock the integral tapering cast steel molds upon the steel ingots. While the molds are made integral and are lifted longitudinally off the solidified ingots, as the so-called osmotic infusion does not take 90 place between the steel of the mold and the steel of the ingot cast therein all danger of the locking of the ingot mold to the ingot is overcome.

I claim:

1. An ingot mold for casting steel composed of cast steel having approximately the same carbon content as that of the steel to be cast therein.
2. An integral ingot mold for casting 100 steel composed of steel containing a carbon content of not over two per cent.
3. A steel ingot mold for casting steel, composed of iron alloyed with carbon, manganese, sulfur and phosphorus, the content 105 of one of the main alloying elements of the mold being not more than two per cent. above the content of the same element of the steel to be poured into the mold.

In testimony whereof, I the said HARRY 110 E. SHELDON have hereunto set my hand.

HARRY E. SHELDON.

Witnesses:

ROBERT C. TOTTEN,  
JOHN F. WILL.